

## UNITED STATES PATENT OFFICE

2,637,687

## ELECTRODEPOSITION OF NICKEL

Lloyd B. Portzer and William C. Leitenberger,  
Cleveland, OhioNo Drawing. Application May 31, 1951,  
Serial No. 229,261

9 Claims. (Cl. 204—49)

1

This invention relates to the electrodeposition of metals and in particular relates to a brightening additive for use in the electrodeposition of bright nickel from a nickel electrolyte.

In the past selection of a brightener for use in the electrodeposition of bright nickel has been predicated upon the same meeting several requirements relative to operability in a standard Watt's bath.

First, it was important that the brightener used be soluble in the entire solution so that the formation of an insoluble precipitate, which would be detrimental to the operation of the bath, would be avoided.

Second, it was important to ascertain that the use of the brightener would not interfere with the action of additional additives used to effectuate separate and distinct functions, such as levelling.

Lastly, it was important that the brightener selected be operable within the entire bath to effectuate a truly lustrous and bright deposit on the article being plated.

Because of the rigidity of the aforementioned requirements, all known brighteners now commercially available on the market, have been found unsatisfactory for one reason or another. Either they were insoluble in the overall bath, interfered with the action of the other additives, or because of these other additives present in the bath, were inoperable to give a truly bright and lustrous plate.

Further difficulty has been encountered in all of the presently available brightening additives in that the same are highly sensitive and accordingly are operable successfully only over a relatively narrow current density range. In practical application, it has been found that if the bath containing the presently available brightening additive is operated outside the aforementioned restricted current density area, the resultant plated product will be characterized by the presence of streaks, which render the product unsatisfactory from a commercial standpoint.

Accordingly, it is one object of this invention to provide a brightening additive which will be soluble in nickel electrolyte over a relatively wide current density range.

It is a further object of this invention to provide a brightening additive which can be made compatible with a levelling additive used in a standard Watt's bath.

It is a further object of this invention to provide a stabilized brightening additive which will not break down under electrolysis to cause the formation of an insoluble precipitate.

2

Other objects of the invention will become apparent upon consideration of the following brief specification and the examples used therein.

Broadly speaking it has been discovered that if a certain class of dye compounds are used in conjunction with certain other chemical compounds, a highly satisfactory brightening additive is formed, which compound satisfactorily meets all the prerequisites previously set forth in this regard.

Specifically, it has been found that if triphenylmethane dyes, and in particular triphenylmethane dyes having an auxochrome group therein, are reduced to the leuco state thereof and then treated with an excess of a holding agent for which the oxygen of the air has a greater affinity than for said reduced leuco compound, the resulting compound will give exceptional results when used as a brightening additive in a Watt's bath. In essence, the foregoing treatment amounts to a reduction to the leuco state by one compound and a holding of the product in that state by another compound. Triphenylmethane dyes which can be satisfactorily treated by this dual process of reduction and holding are listed in table A below.

TABLE A

1. Fuchsine
2. Pararosaniline
3. Rosaniline
4. Methyl Violet
5. Aniline Blue
6. Iodine Green
7. Aurine
8. Acid Fuchsin

The underlying theory for this dual process of reduction and holding stems from the discovery that a relatively rapid reduction of the triphenylmethane dye to the leuco state changes the dye from an insoluble compound to a soluble compound capable of use in an electroplating bath. Further treatment in the form of use of a compound which will hold this first mentioned compound in the leuco state is necessitated by the fact that unless so treated, the leuco compound will gradually oxidize and revert to the original insoluble dye product, and accordingly be unsatisfactory for use in the bath. Experimentation has shown that the use of zinc powder and hydrochloric acid is satisfactory to reduce the dye to the leuco state if the amounts used are controlled so that the triphenylmethane dye would not be reduced to the point where an excess of this reducing agent was present in the form of an insoluble precipitate which would

disadvantageously affect the results obtained from the plating solution. Hence it became manifest that further oxidation that would normally take place must be prevented, or at least compensated for, by the use of compound which would not result in the formation of an insoluble precipitate that would act to destroy the overall solubility of the brightening additive. Best results in this regard could be obtained by using an oxygen containing compound for which the oxygen possessed a greater affinity than for the reduced leuco compound. In practical application, it was found that use of either sodium hydrosulphite or sodium bisulphite was satisfactory to effectuate the desired holding action, inasmuch as the addition of an excess amount of either one of these compounds did not result in the creation of an insoluble precipitate.

While all of the compounds listed in Table A can be satisfactorily treated as just described, it has been found that certain of the compounds are soluble in the nickel electrolyte without the presence of the reducing and holding agents and accordingly the use of these soluble compounds per se is intended to be within the scope of this invention.

In practice, satisfactory brightening additives for use in the newly discovered process have been prepared by employing the mixture of each of the below listed examples:

*Example 1*

|                      |       |     |
|----------------------|-------|-----|
| Pararosaniline       | grams | 450 |
| Zinc powder          | do    | 120 |
| Hydrochloric acid    | cc    | 200 |
| Sodium hydrosulphite | pound | 1   |
| Water                | gal   | 13  |

*Example 2*

|                      |       |     |
|----------------------|-------|-----|
| Rosaniline           | grams | 454 |
| Zinc powder          | do    | 120 |
| Sulfuric acid        | cc    | 100 |
| Sodium hydrosulphite | pound | 1   |
| Water                | gal   | 13  |

*Example 3*

|                      |       |     |
|----------------------|-------|-----|
| Methyl Violet        | grams | 450 |
| Zinc powder          | do    | 120 |
| Sulphuric acid       | cc    | 100 |
| Sodium hydrosulphite | pound | 1   |
| Water                | gal   | 13  |

*Example 4*

|                      |       |     |
|----------------------|-------|-----|
| Fuchsin              | grams | 454 |
| Zinc powder          | do    | 120 |
| Sulphuric acid       | cc    | 100 |
| Sodium hydrosulphite | pound | 1   |
| Water                | gal   | 13  |

*Example 5*

|                      |       |     |
|----------------------|-------|-----|
| Aniline Blue         | grams | 448 |
| Zinc powder          | do    | 120 |
| Hydrochloric acid    | cc    | 200 |
| Sodium hydrosulphite | pound | 1   |
| Water                | gal   | 13  |

*Example 6*

|                   |       |     |
|-------------------|-------|-----|
| Iodine Green      | grams | 450 |
| Zinc powder       | do    | 120 |
| Sulphuric acid    | cc    | 100 |
| Sodium bisulphite | pound | 1   |
| Water             | gal   | 13  |

*Example 7*

|                     |       |     |
|---------------------|-------|-----|
| Aurine              | grams | 450 |
| Zinc powder         | do    | 120 |
| Hydrochloric acid   | gal   | 1/2 |
| 5 Sodium bisulphite | pound | 1   |
| Water               | gal   | 13  |

NOTE.—The designation of weights employed in the above examples relate only to amounts used in preparing the brightening additive per se, and in no way relate to volumes used in plating baths. In practice, each of the above additives, shown by a specific example, constitutes approximately 0.1-0.2% of the volume of the plating tank.

Thus it will be seen that use of triphenylmethane dye in conjunction with a reducing agent and a holding agent will result in a brightening additive having the desirable property of being compatible with other additives over a relatively wide current density range.

For the purpose of illustrating how the brightening additives set forth in the above described examples may be satisfactorily utilized to commercially electrodeposit bright nickel, certain electrolytic solutions which have been found to be satisfactory, are described in the below-listed examples.

*Example 8*

|                           |                 |
|---------------------------|-----------------|
| Nickel sulphate           | 40 oz./gal.     |
| Nickel chloride           | 8 oz./gal.      |
| Boric acid                | 6 oz./gal.      |
| Brightening additive (Per |                 |
| Example #2)               | .15% by volume. |

pH 4.0.

Temperature 135°-145° F.

Current density 50 amps./sq. ft.

*Example 9*

|                           |             |
|---------------------------|-------------|
| Nickel sulphate           | 45 oz./gal. |
| Nickel chloride           | 8 oz./gal.  |
| Boric acid                | 6 oz./gal.  |
| Brightening additive (Per |             |

Example #1) .15% by volume.

pH 4.5.

Temperature 135°-145° F.

Current density 50 amps./sq. ft.

*Example 10*

|                           |             |
|---------------------------|-------------|
| Nickel sulphate           | 50 oz./gal. |
| Nickel chloride           | 10 oz./gal. |
| Boric acid                | 5 oz./gal.  |
| Brightening additive (per |             |

Example #3) .20% by volume.

pH 4.5.

Temperature 135°-145° F.

Current density 35 amps./sq. ft.

*Example 11*

|                           |             |
|---------------------------|-------------|
| Nickel sulphate           | 40 oz./gal. |
| Nickel chloride           | 8 oz./gal.  |
| Boric acid                | 6 oz./gal.  |
| Brightening additive (per |             |

Example #4) .20% by volume.

pH 4.5.

Temperature 135°-145° F.

Current density 35 amps./sq. ft.

It follows that modifications of the invention and further combinations under the above examples may be resorted without deviating from the spirit thereof and the scope of the appended claims.

What is claimed is:

1. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and hydrochloric acid, and

a holding agent selected from the group consisting of sodium bisulfite and sodium hydrosulfite.

2. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and sulfuric acid, and a holding agent selected from the group consisting of sodium bisulfite and sodium hydrosulfite.

3. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and hydrochloric acid and a holding agent comprising sodium bisulfite.

4. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and hydrochloric acid, and a holding agent comprising sodium hydrosulfite.

5. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and hydrochloric acid, and a holding agent selected from the group consisting of sodium bisulfite and sodium hydrosulfite.

6. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and hydrochloric acid, and a holding agent selected from the group consisting of sodium bisulfite and sodium hydrosulfite.

presence of a reduced triphenylmethane dye obtained by the reaction of the corresponding triphenylmethane dye with a reducing agent comprising zinc powder and a mineral acid, and a holding agent selected from the group consisting of sodium bisulfite and sodium hydrosulfite.

5 7. A method of electrodepositing nickel from a nickel electrolyte comprising an aqueous acid solution of a nickel salt, comprising the step of electrolyzing said nickel electrolyte in the presence of a reduced triphenylmethane dye obtained by the reaction of the corresponding triphenylmethane dye with a reducing agent comprising zinc powder and a mineral acid, and a holding agent selected from the group consisting of sodium bisulfite and sodium hydrosulfite.

10 8. A bath for electrodepositing nickel from a nickel electrolyte comprising an aqueous acid solution of a nickel salt comprising, a nickel electrolyte and a reduced triphenylmethane dye obtained by the reaction of the corresponding triphenylmethane dye with a reducing agent comprising zinc powder and hydrochloric acid, and a holding agent selected from the group consisting of sodium bisulfite and sodium hydrosulfite.

15 9. A bath for electrodepositing nickel from an aqueous acid solution of a nickel salt comprising, an aqueous acid solution of a nickel salt and a reduced triphenylmethane dye obtained by the reaction of the corresponding triphenylmethane dye with a reducing agent comprising zinc powder and hydrochloric acid, and a holding agent selected from the group consisting of sodium bisulfite and sodium hydrosulfite.

20 35 LLOYD B. PORTZER.  
WILLIAM C. LEITENBERGER.

References Cited in the file of this patent

UNITED STATES PATENTS

40 Number Name Date  
2,198,268 Lind et al. Apr. 23, 1940

OTHER REFERENCES

American Dyestuff Reporter, November 1, 1948,  
45 pp. 709, 720, 723, and 724.